

Aug. 5, 1958

R. C. BUCHAN

2,846,385

PREVENTION OF CORROSION IN WELLS

Filed Oct. 11, 1954



INVENTOR.  
Rudolph C. Buchan,  
BY

*Rudolph C. Buchan*  
ATTORNEY.

1

2,846,385

## PREVENTION OF CORROSION IN WELLS

Rudolph C. Buchan, Houston, Tex., assignor, by mesne assignments, to Esso Research and Engineering Company, Elizabeth, N. J., a corporation of Delaware

Application October 11, 1954, Serial No. 461,566

5 Claims. (Cl. 204—148)

The present invention is directed to a method for preventing corrosion in wells. More particularly, the invention is concerned with protecting a steel well casing from corrosion by corrosive well fluids. In its more specific aspects, the invention is directed to a method for protecting a steel well casing from corrosion by corrosive well fluids forming a stagnant body in the casing.

The present invention may be briefly described as a method for protecting a steel well casing from corrosion by corrosive well fluids in contact therewith in which a tubing is arranged having its lower open end at a level a substantial distance above a zone from which said corrosive well fluids are produced. A stagnant body of said corrosive well fluids is in contact with the steel casing. The method particularly comprises lowering a retrievable, sacrificial-metal tubular member, smaller in diameter than the tubing, through the tubing until the tubular member projects a substantial distance from the lower open end of the tubing and extends from the open end of the tubing to the zone from which the corrosive well fluids are produced. The sacrificial metal tubular member is anodic to steel and is electrically connected to the tubing. The tubular member is maintained in the tubing and casing while the corrosive fluids are produced such that the casing is protected from corrosion by the corrosive fluids and the tubular member is corroded instead.

The sacrificial metal making up the tubular member may be zinc, magnesium, aluminum and/or alloys of these materials, and the like.

The invention contemplates the removal of the tubular member periodically from the tubing, while the tubing remains in place, for determination of the extent of corrosion taking place in the well. The corrosive nature of the well fluids will be indicated by corrosion of the sacrificial metal and is further contemplated that as the sacrificial metal tubular member is corroded it may be replaced by another tubular member of a metal anodic to steel.

The present invention will be further illustrated by reference to the drawing in which the single figure discloses apparatus illustrating a preferred mode.

Referring now to the drawing, numeral 11 designates a well bore drilled in the earth to penetrate a plurality of hydrocarbon productive intervals 12, 13, and 14 which may be separated from each other by non-productive intervals of zones 15 and 16.

In this particular instance, the well bore 11 has a steel casing 17 arranged therein which is cemented in place with primary cement 18. The casing 17 has a tubing 19 arranged therein with its lower open end 20 above the hydrocarbon productive interval 12. There is provided, for closing the annulus A between the casing 17 and the tubing 19 a packer 21 which may be a packer such as illustrated in the 20th edition of the Composite Catalog on pages 875 and 876 or on pages 496 and 497 of the catalog, supra, which illustrated

2

packers of the catalog, supra, comprise means for establishing a metal-to-metal contact between the casing 17 and the tubing 19. In the drawing a packer of the type illustrated on pages 875 and 876 of the catalog, supra, is schematically shown, such packer comprising upper and lower expandable cup members 1 and 2 fixed to retaining rings 3 and 4, respectively. The retaining ring 3 is slidable with respect to the tubing 17 and is inwardly, downwardly tapered against the lower end thereof for bearing engagement with slips 5 to force such slips 5 into engagement with the casing 17, as shown. A stagnant zone Z of corrosive well fluids thus exists below the packer 21 which may rapidly corrode the casing.

15 In the practice of the present invention, an elongated tubular member 22 is lowered through the tubing 19, such as on a wire line, not shown, and secured and/or supported in a landing nipple, such as 22a, which may be a landing nipple, such as described in the Composite Catalogue, supra, at page 4000. The tubular extension member 22 which is constructed of sacrificial metal of the nature described supra is electrically connected to the tubing 19 by means 23 which may comprise the landing nipple 22a but which will include a suitable metal to 20 metal bond. The tubular extension member 22 extends with its lower end to the perforations 24 which were formed in the casing 17 to perforate the hydrocarbon productive interval or zone 14 to allow production of corrosive 25 fluids which may include hydrocarbons and salt water. The salt water may be corrosive due to the presence of corrosive salts, sulfides, such as hydrogen sulfide, metal sulfides, and the like, and due to the presence of organic acids, and carbon dioxide, and the like. The corrosive 30 fluids including hydrocarbons ordinarily will proceed upwardly through the tubular member 22 and upwardly through the tubing 19 following the path described by the arrows and to a zone Z where a relatively stagnant body of corrosive well fluids will exist which will corrode 35 the casing 17.

In accordance with the present invention, with a sacrificial metal tubular member 22 of the nature described supra anodic to the steel casing 17 extending from the tubing 19, the steel casing 17 is not corroded by corrosive 40 fluid in the zone Z above the lower end of the tubular member 22 and the sacrificial metal tubular member 22 is corroded, thereby protecting the casing 17 from corrosion.

From time to time the tubular member 22 may be 45 retrieved from the tubing 19 while the tubing 19 is maintained in place and the tubular member 22 withdrawn to the well head by engaging the fishing neck 25 with a fishing tool carried on a wire line, not shown, and the extent of corrosion of the tubular member 22 determined

50 by inspection. The inspection will also reveal the corrosiveness of the corrosive fluid in the zone Z. If it is determined that corrosion is being suffered by the corrodible tubular member 22 to the extent that its utility is destroyed, the tubular member 22 may be replaced by 55 another sacrificial metal tubular member constructed of a metal anodic to a steel casing 17.

It may be seen from the foregoing description taken with the drawing that the present invention is of great utility in that protection of steel casing is provided without resort to introduction of chemicals, such as inhibitors and the like, into the well.

60 The tubular member 22 has been described as being constructed of sacrificial metal, such as magnesium, zinc, or aluminum. It is contemplated that the tubular member 22 need not be constructed throughout its total length of the sacrificial metal but may be constructed of sections 65 of sacrificial metals, such as zinc, magnesium, or alumi-

num, as desired. However, it would be preferred to construct the tubular member 22 of the sacrificial metal due to its lightness and due to ease in manipulation and protection of the casing 17.

The nature and objects of the present invention having been completely described and illustrated, what I wish to claim as new and useful and to secure by Letters Patent is:

1. A method for protecting a portion of a steel well casing adjacent a hydrocarbon producing formation from corrosion by a stagnant body of corrosive fluids accumulated in said portion of said casing by production from said formation into said casing, said casing having a tubing arranged therein with the lower end of said tubing above said stagnant body of corrosive fluids in said portion of said casing, which method comprises the steps of metallically, annularly interconnecting said tubing with said casing adjacent said lower end of said tubing to thereby establish an electrical interconnection between said casing and said tubing adjacent said lower end of said tubing, lowering a retrievable sacrificial metal tubular member smaller in diameter than said tubing through said tubing until said tubular member projects a substantial distance from the lower end of said tubing and extends to said portion of said casing containing said corrosive well fluids, said sacrificial metal being anodic to steel, whereby a galvanic action is established in said portion of said casing adjacent said producing formation, and maintaining said tubular member in said tubing and casing while said corrosive fluids are produced, whereby said portion of said casing is protected from corrosion by said corrosive fluids and said sacrificial member is corroded.

2. A method in accordance with claim 1 wherein the sacrificial metal is zinc.

3. A method in accordance with claim 1 wherein the sacrificial metal is magnesium.

4. A method in accordance with claim 1 wherein the sacrificial metal is aluminum.

5. A method for protecting a portion of a steel well casing adjacent a hydrocarbon producing formation from corrosion by a stagnant body of corrosive fluids accumulated in said portion of said casing by production from said formation into said casing, said casing having a tubing arranged therein with the lower end of said tubing above said stagnant body of corrosive fluids in said portion of said casing, which method comprises the steps of closing the annulus between said tubing and said casing adjacent the lower end of said tubing and metallically, annularly interconnecting said tubing with said casing adjacent said lower end of said tubing to thereby establish an electrical interconnection between said casing and said tubing adjacent said lower end of said tubing, lowering a retrievable sacrificial zinc tubular member smaller in diameter than said tubing through said tubing until said tubular member projects a substantial distance from the lower end of said tubing and extends to said portion of said casing containing said stagnant body of said corrosive well fluids, whereby a galvanic action is established in said body of said casing adjacent said producing formation, and maintaining said tubular member in said tubing and casing while said corrosive fluids are produced, whereby said portion of said casing is protected from corrosion by said corrosive fluids and said sacrificial member is corroded.

References Cited in the file of this patent

UNITED STATES PATENTS

|    |           |               |       |               |
|----|-----------|---------------|-------|---------------|
| 30 | 1,608,709 | Mills         | ----- | Nov. 30, 1926 |
|    | 1,804,078 | Baden         | ----- | May 5, 1931   |
|    | 2,149,617 | Menaul        | ----- | Mar. 7, 1939  |
|    | 2,155,370 | Hall et al.   | ----- | Apr. 18, 1939 |
| 35 | 2,244,322 | Zoller et al. | ----- | June 3, 1944  |
|    | 2,401,546 | Brown         | ----- | June 4, 1946  |
|    | 2,665,759 | Childers      | ----- | Jan. 12, 1954 |

FOREIGN PATENTS

|    |         |               |       |               |
|----|---------|---------------|-------|---------------|
| 40 | 523,618 | Great Britain | ----- | July 19, 1940 |
|----|---------|---------------|-------|---------------|